# EUROPEAN PATENT SPECIFICATION

(11) **EP 0 150 549 B1**
(45) Date of publication and mention of the grant of the patent: **12.07.1989**
(21) Application number: 84300619.8
(22) Date of filing: 01.02.1984
(51) Int. Cl.: B22D 11/10, B22D 41/08

(54) **Nozzle for continuous casting**
Düse für das Stranggiessen
Tuyère pour la coulée continue

(43) Date of publication of application: 07.08.1985
(73) Proprietor: Akechi Ceramics Kabushiki Kaisha, Ena-gun Gifu-ken (JP)
(72) Inventor: Kondo, Masanao, Ena-gun Gifu-ken (JP)
(74) Representative: Waite, Anthony William

(56) References cited:
- WO-A-84/04893
- DE-A- 2 527 585
- DE-A- 2 822 518
- DE-A- 3 216 478
- DE-B- 2 936 480
- DE-C- 3 149 399

## Description

This invention relates to a nozzle for continuous casting.

Hitherto a gas blow-in type nozzle for continuous casting has been known wherein an inert gas is blown in to an inner surface of the nozzle through the nozzle body so as to form a gas seal on the inner wall surface and prevent the nozzle from clogging.

As shown in Figures 1 and 2 of the accompanying drawings, an example of this kind of nozzle has an annular gap formed in a wall thereof, said gap forming a gas pressure balance chamber 2 which is connected via a gas inlet hole 3 to an inert gas supply source disposed outside the nozzle body 1 whilst communicating with the inner surface of the nozzle body via open pores existing therein, whereby the inert gas is made to blow into the space between the inner wall surface and the molten steel. Such a gap is made by using a solid material such as will disappear during the burning process for manufacturing a nozzle, for example, paper, polypropyrene, nylon paraffin, etc. The gap is made by providing said material in an appropriate place inside the nozzle body wall at the time of moulding and thereafter burning it away.

Another example of the aforesaid kind of nozzle having an annular gap formed in a wall thereof into which gas is introduced via a passage communicating with the exterior, is disclosed in DE-A-2822518.

The open pores which communicate the gas pressure balance chamber 2 with the inner surface of the nozzle are naturally formed during the nozzle manufacturing process so that the existence of the open pores is not always uniform and varies according to the manufacturing conditions. Therefore, there has arisen a problem that the amount of gas supplied to the inner surface is not constant or uniform. In particular, when the number of open pores of less than 5 pm in diameter present is more than 50% in the prior art nozzle, it is practically difficult to blow in the gas and impossible to form a perfect gas seal.

A further prior nozzle of the aforesaid general kind is shown in Figures 11 and 12 of WO 84/04893, an Article 54(3) document, from which the single claim starts, in which gas is introduced from the exterior into an annular gap in the wall thereof and thence into the nozzle interior through an array of holes having a diameter between 0.2 and 0.5 mm.

An object of the invention is to provide an improved gas blow-in type nozzle for continuous casting in which the foregoing disadvantages are alleviated or avoided, the nozzle of the invention leading to improved uniformity of gas supply to the nozzle inner wall and having a reduced tendency to clogging.

In the nozzle of the invention, each hole through which the pressure balance chamber communicates with the inner wall surface of the passageway has an area corresponding to that of a circular hole having a diameter of 0.03 to 0.05 mm., and the nozzle body has a maximum porosity of 20% whilst containing at least 50% of open pores each having a maximum diameter of 5 pm.

In the accompanying drawings,
Figures 1 and 2 are vertical sectional views showing conventional nozzles, and
Figures 3 and 4 are vertical sectional views showing, by way of example, nozzles according to the present invention.

### Detailed Description of the Embodiments

Referring to Figs. 3 and 4, a nozzle body 10 has a slit-form gap or gas pressure balance chamber 11 which is disposed in an appropriate place inside the nozzle body 10. A gas inlet hole 12 is formed inside the nozzle body 10 so as to connect the gas pressure balance chamber 11 to an inert gas supply source disposed outside the nozzle. Numeral 13 indicates a slag line portion. A plurality of communication holes 14 are formed in the longitudinal and diametrical directions of the nozzle body 10 at appropriate intervals so as to communicate the gas pressure balance chamber to the inner wall surface of the nozzle body 10. Each communication hole is 0.03 to 0.5 mm in diameter depending upon the penetration of the molten steel to the communication hole 14 when the inert gas is not blown in. The best-suited sectional shape of the communication hole is a circular one for the purpose of preventing the occurrence of the structural defects of the nozzle, but of course it is to be noted that the sectional shape of the communication hole 14 must not be limited thereto and may be in any shape whatever as long as the area of the hole corresponds to that of a circular hole within the scope of the aforementioned size. The present invention is most effective when the nozzle body is mainly made of generally known natural graphite and various kind of alumina, sintered alumina, a-alumina, P-atumina, high-alumina materials (mullite, sillimanite, etc.) and chemically composed of 10% to 40% carbon, 40% to 80% alumina and 20% or less silica, etc., with the use of synthetic resin bond as a bonding agent.

The present invention will be explained hereinbelow with reference to the preferable examples.

### Example 1

When simultaneously using the two immersion nozzles shown in Table 1 for pouring AI-killed steel of Sol-Al 0.070% with ladle having a capacity of 250 ton, the present nozzle was capable of perfectly pouring eight ladles without any adhesion of A1₂0₃ while the conventional nozzle was adhered with A1₂0₃ when it poured five ladles and incapable of further casting. Thus the remarkable effects of the present nozzle have been confirmed.

### Example 2

When simultaneously using the two immersion nozzles shown in Table 2 for pouring AI-killed steel of Sol-AI 0.05% with ladle having a capacity of 300 ton, the present nozzle was capable of perfectly pouring seven ladles without any adhesion of AI₂0₃ while the conventional nozzle was adhered with Al₂O₃ when it poured four ladles and incapable of further casting. Thus the remarkable effects of the present nozzle have been confirmed.

As seen from the above, the immersion nozzle according to the present invention was capable of continuous casting without clogging up, as compared with the conventional one.

## Claims

A nozzle for continuous casting comprising a nozzle body (10) having a wall defining a central passageway, and a gas pressure balance chamber (11) formed in said wall and communicating with the exterior via a passage (12), said chamber (11) communicating with the inner wall surface of the passageway by way of a plurality of holes (14), wherein each hole (14) has an area corresponding to that of a circular hole having a diameter of 0.03 to 0.5 mm., and said nozzle body (10) has a maximum porosity of 20% and contains at least 50% of open pores each having a maximum diameter of 5 µm.

## Patentansprüche

Düse zum kontinuierlichen Gießen mit einem Düsenkörper (10), der eine Wand besitzt, die einen Zentralen Kanal definiert, mit einer Gasdruck-Augsgleichskammer (11), die in der Wand ausgebildet ist und über einen Durchlaß (12) mit der äußeren Umgebung in Verbindung steht, wobei die Kammer (11) mit der Innenfläche der Wand des Kanals über mehrere Öffnungen (14) in Verbindung steht, bei welcher (nämlich bei der Düse) jede Öffnung (14) eine Fläche hat, die derjenigen einer kreisrunden Öffnung mit einem Durchmesser von 0,03 bis 0,5 mm entspricht, und der Düsenkörper (10) eine maximale Porosität von 20% besitzt und mindestens 50% von offenen Poren hat, von denen jede einen maximalen Durchmesser von 5 pm besitzt.

## Revendications

Tuyère pour la coulée en continu, comprenant un corps de tuyère (10) possédant une proi définissant une voie de passage centrale, et une chambre e'équilibrage de pression de gaz (11) formée dans cette paroi et communiquant avec l'extérieur par l'intermédiaire d'un passage (12), la chambre (11) communiquant avec la surface de paroi intérieure de la voie de passage au moyen d'une pluralité d'orifices (14), dans laquelle chaque orifice (14) a une superficie correspondant à celle d'un orifice circulaire d'un diamètre de 0,03 à 0,5 mm, et le corps de tuyère (10) a une porosité maximale de 20% et contient au moins 50% de pores ouverts présentant chacun un diamètre maximal de 5 µm.
